

# UNITED STATES PATENT OFFICE.

WILLIAM BEACH PRATT, OF WELLESLEY, MASSACHUSETTS, ASSIGNOR TO E. H. CLAPP RUBBER COMPANY, OF BOSTON, MASSACHUSETTS, A CORPORATION OF MASSACHUSETTS.

## WATERPROOFED FABRIC.

1,349,910.

Specification of Letters Patent. Patented Aug. 17, 1920.

No Drawing. Application filed January 8, 1919, Serial No. 270,228. Renewed May 3, 1920. Serial No. 378,660.

*To all whom it may concern:*

Be it known that I, WILLIAM BEACH PRATT, a citizen of the United States, residing at Wellesley, in the county of Norfolk and State of Massachusetts, have invented new and useful Improvements in Waterproofed Fabrics, of which the following is a specification.

This invention has for its object the production of a fabric which is resistant to oxidation, capable of vulcanization onto rubber, and waterproofed, so that it may be used for a great variety of purposes in the art, such as in the manufacture of rubber tires, shoes, belting, hot water bottles, packing, rain-coats, filter cloth, carriage tops, waterproof coverings, paulins, etc.

A fabric, embodying the present invention, consists of a fibrous body or foundation treated with a non-colloidal sulfur-terpene compound, in which the fibers are saturated or impregnated with the compound and thereby are rendered resistant to rotting or disintegration when subjected to the elements. The fibrous body or foundation may consist of a thread, cord or rope, either single or interwoven or braided with others in the form of a cloth or braid, or it may consist of a sheet or other fabricated form in which the fibers are interlocked or felted.

This foundation is treated with the suitable sulfur-terpene compound while the latter is in a liquid state, that is, either when thinned by a suitable solvent or rendered liquid by the application of heat.

The impregnating or converting compound should be non-colloidal so that it will tend to penetrate the fibers of the foundation, as well as coat them, and it should be of such oxidation-resistant character that it will safeguard the fibers from rotting and disintegration, and will render them water and weather proof. Furthermore such compound should be neutral, *i. e.* neither acid nor alkaline, and should be capable of being united to rubber and rubber compounds by vulcanization.

I have found that, by the digestion of certain terpenes (for example, oil of turpentine,) with sulfur in a reflux condenser under proper thermal conditions, a neutral amorphous non-colloidal sulfur compound is produced which may be employed in the

production of a fabric embodying the present invention. In preparing such compound, oil of turpentine and sulfur, in the ratio of about 2 to 1.5 parts by weight, (or if desired, in equal parts) are digested with a reflux condenser at a temperature of 140° C. or above, and the reaction is continued until the mass on cooling is a solid or semi-solid as desired, the reaction being progressive and the sulfur combining with the turpentine, with the liberation of hydrogen sulfid. The time of treatment depends upon the desired consistency of the product, the temperature, and whether the mass undergoing digestion is agitated. I do not herein claim either the sulfur-terpene compound, or the process of producing it. When the reaction is carried to completion, the resulting product, *i. e.* the sulfur-terpene compound, is a hard tough black mass, breaking with a conchoidal fracture, presenting a vitreous luster on the surfaces of the fracture. It is soluble in turpentine with reaction, partly soluble in acetone, soluble in toluol and in xylol, and insoluble in water. A portion of this mass, when manipulated between the fingers, will, under the heat of the hand, become so softened that it can be molded.

In the production of a fabric embodying the invention, I preferably dry, by the application of moderate heat, the fibrous foundation to eliminate moisture therefrom (though this step is not essential), and then I either immerse the fabric in a bath of the liquid compound, or coat the latter thereon. The sulfur-terpene compound is preferably thinned by a suitable solvent so that it will quickly penetrate the fibers and the interstices between them, but under some circumstances I heat the compound to a liquid or plastic condition and apply it as a paint. For treating cloth, thread, felt or other fabrics, a satisfactory solution may be prepared by dissolving 1 part by weight of sulfur-terpene compound in 4 parts by weight of xylol under mild heat. After the fabric has been impregnated therewith, the fabric is subjected to sufficiently elevated temperatures to drive off the solvent in a reasonable time, or, if desired, it is subjected to vacuum drying for more complete recovery of the solvent, according to common practice.

- One of the great advantages of a fabric impregnated with a sulfur-terpene compound, as herein described, is that it possesses a tensile strength that could not have been predicated on the strength of the original fiber. For example, a "17.5 ounce auto. fabric," such as is commonly employed in the construction of pneumatic tires, when made from short staple American cotton, 10 has been increased in strength, by impregnation with said sulfur-terpene compound, to that of a similar untreated fabric made of Egyptian cotton. Such fabrics produced from higher grades of American cotton, or 15 of Egyptian cotton, when so impregnated surpass in strength any similar untreated fabric made of any grade of cotton whatever.
- Likewise such fabrics or fabricated forms, 20 as threads, sheets formed of interlocked threads (*i. e.* woven, knitted or braided), paper or paper felt, etc. when treated with the sulfur-terpene compound are increased in strength to a marked degree.
- 25 Another of the great advantages of a material such as herein described is that it will vulcanize onto and with rubber, and thus it may be employed in the manufacture of all kinds of rubber goods. For example, 30 if the foundation consists of a woven fabric, treated as described, it may be surfaced on one or both faces with a thin layer of rubber compound and be used in the construction of hot water bags or fountain syringes,
- 35 which will greatly outwear those as now commercially manufactured. The protection, which the compound affords to the fibers, prevents their rotting and disintegrating when exposed to air, water, or weak 40 acids or alkalis, and makes it possible to employ the material herein described for a great variety of uses.
- It has heretofore been common practice, 45 when a cord or sheet of fibrous material is to be used with rubber compounds in the manufacture of rubber articles, to "friction" the same with a rubber coating in order to press the rubber into the interstices or meshes of the fibrous material, and permit the vulcanization of the fabric so "frictioned" with adjacent layers or masses of rubber compound. The rubber, which is frictioned into the fabric, does not protect 50 the fibers thereof, if the rubber coating is worn or separates therefrom, and consequently the fibers are liable to rapid oxida-

tion and disintegration. Moreover, the mechanical manipulations in the operation of frictioning rubber into fabric must be carried out under most exacting conditions, for 60 there is always a danger of injuring the fibers and impairing the strength of the fabric, due to the pressure requisite to press or mechanically force the rubber into the meshes or interstices of the fabric. 65

A fabric embodying my invention has none of these disadvantages, for the sulfur-terpene compound, being non-colloidal, will soak in or penetrate the fibers and become absorbed without mechanical pressure, and 70 the strength of the fabric is greatly increased, as hereinafter pointed out. Each fiber may be coated with a film of the compound which is capable of vulcanization to rubber, and a greater contact between the 75 rubber and the fabric is therefore afforded than is possible with "friction" cloth or fabric.

I do not claim herein either the herein 80 described sulfur-terpene compound, or the process of making the same, since they form the subject-matter of my co-pending application Serial No. 328,235, filed October 3, 1919.

Having thus explained the nature of my 85 said invention, and described a way of making and using the same, although without attempting to set forth all of the forms in which it may be made or all of the modes of its use, what I claim is:—

1. A fabric consisting of a fibrous foundation impregnated with a non-colloidal sulfur-terpene compound.
2. A fabric consisting of a fibrous thread impregnated with a non-colloidal sulfur-terpene compound.
3. A fabric consisting of a plurality of interlocked threads impregnated with a non-colloidal sulfur-terpene compound.
4. The herein described process which 100 consists in permeating the fibers of a fibrous material with a non-colloidal sulfur-terpene compound.
5. The herein described process which 105 consists in impregnating the fibers of a fibrous material with a solution containing a non-colloidal sulfur-terpene compound, and then removing the solvent.

In testimony whereof I have affixed my signature.

WILLIAM BEACH PRATT.